

Oct. 3, 1933.

A. H. IRVING ET AL

1,929,279

PAVEMENT

Filed Feb. 24, 1931



INVENTORS  
ANDREW H. IRVING  
OWEN H. ROBERTSON  
BY *Charles S. Evans*  
THEIR ATTORNEY

## UNITED STATES PATENT OFFICE

1,929,279

## PAVEMENT

Andrew H. Irving, Berkeley, and Owen H. Robertson, Oakland, Calif., assignors to The Paraffine Companies, Inc., San Francisco, Calif., a corporation of Delaware

Application February 24, 1931. Serial No. 517,754

2 Claims. (Cl. 94—5)

Our invention relates to a pavement, and particularly to improvements in the wear-taking layer of a paving structure which possesses the property of "healing" over minor injuries inflicted in its surface, such as that described in the patent to William H. Lowe, No. 1,610,019, patented Dec. 7, 1926.

It is among the objects of our invention to provide a pavement which is possessed of great durability together with a certain measure of resilience coupled with vibration absorbing and sound deadening properties.

Another object of our invention is the provision, in a pavement of the character described, of a wear-taking layer which presents a skid-proof traction surface.

Another object of our invention is the provision, in a pavement of the character described, of means for reducing the resistance to trucking.

A further object of our invention includes the provision, in a pavement of the character described, of means for accomplishing the above mentioned objects without impairing the "healing" properties of the traffic sheet, as set forth in the patent previously referred to.

The invention possesses other objects and features of advantage, some of which, with the foregoing, will be set forth in the following description of our invention. It is to be understood that we do not limit ourselves to this disclosure of species of our invention, as we may adopt variant embodiments thereof within the scope of the claims.

35 Referring to the drawing:

The figure of the drawing is a perspective view showing a portion of the pavement embodying our invention. Part of the finishing coating is omitted to show more clearly the character of the wear-taking layer surface.

In connection with paving structures it is difficult to over-estimate the value of a traffic sheet having a wear-taking layer of viscous material slightly and slowly flowable under pressure to render it capable of coalescing after scarring, so that a continuous smooth surface is restored by wear. Possessed of this "self-healing" property a wear-taking layer soon fills up and heals over minor mechanical injuries inflicted by the wearing action of heavy shoes, falling objects, vehicular traffic and other destructive agencies.

When a wear-taking layer of this sort is provided as a coating over a base layer having a certain measure of resilience, such as a fibrous layer saturated with a semi-solid material, a

traffic sheet is provided which is characterized by extreme durability; in actual tests it having been found that the sheet will outwear a steel plate. Accompanying the advantages that flow from this traffic sheet however are certain inherent disadvantages.

The first of these is the fact that the material in the wear-taking layer tends to flow out under the pressure of a load and "hill-up" ahead of a moving truck wheel. The effect of this is to materially increase the resistance to trucking, because a truck is constantly having to climb over a small hill of material. The second disadvantageous feature lies in the fact that the wear-taking layer becomes slippery when wet; this factor being accompanied by a decrease in traction and increased danger to traffic.

The broad object of our invention is to improve a paving structure of the general character described by providing a traffic sheet having a wear-taking layer possessed of the "self-healing" properties pointed out, which materially reduces the resistance to trucking, and which presents a skid-proof traction surface.

In terms of broad inclusion, the pavement embodying our invention comprises a traffic sheet overlying and preferably united with a supporting substructure. The traffic sheet comprises a wear-taking layer of viscous material slightly and slowly flowable under pressure to render it capable of coalescing after scarring, so that a continuous smooth surface is restored by wear. This wear-taking layer is filled with a stiffening material to prevent the flowable material from hill-ing-up under a rolling load, and without impairing the surface restoring properties of the layer.

The filling material is preferably of a granular nature, such as sand; it having been found that such material preserves the "self-healing" properties of the wear-taking layer, and at the same time materially reduces its resistance to trucking. Furthermore, the granular filled layer presents a non-skid traction surface. The viscous material of the wear-taking layer is preferably a bituminous material solid at ordinary temperatures but capable of coalescing after scarring, and is preferably applied as a coating on a preferably resilient base layer. This base layer is preferably a fibrous layer saturated with a semi-solid material. The base layer and wear-taking layer form an integral mass, and this traffic sheet is preferably adhesively united with the supporting substructure, so that a unitary paving structure is provided.

In greater detail, the preferred form of pavement embodying the improvements of our invention comprises a traffic sheet overlying and preferably united with a supporting substructure, such as the concrete foundation 2. The bond between the traffic sheet and substructure is preferably secured by a layer 3 of adhesive, such as a bituminous cement. A relatively hard steam blown asphalt dissolved in carbon bisulfide, benzole, or other suitable solvent may be used in the bonding layer 3; it being understood however that other means may be employed to unite the traffic sheet with the substructure.

A layer 4 of resilient material is preferably provided adjacent the substructure 2, and comprises the base layer of the traffic sheet. We have found it convenient and satisfactory to make the base layer 4 of fibrous material, such as a felt ranging from 35 to 70 lbs. per 480 square feet. The furnish for this felt may be of any suitable material, such as for example a furnish comprising 10% old newspapers, 15% wool rags, 10% burlap and 65% cotton rags. If desirable, a filler, such as wood sawdust or the like, may be added to the furnish. The stock is preferably beaten very short, for such a weight of felt, and is preferably well jordaned.

In order to give body and strength to the fibrous layer, and at the same time render it waterproof and protect it against deterioration, the base layer is preferably treated with a suitable saturant. Furthermore, in order to give the treated fibrous layer a certain measure of resilience, the base layer is preferably saturated with a semi-solid material. A bituminous saturating compound, such as a good grade of soft blown asphalt having a softening point of from 120° to 125° and a penetration of from 50 to 80, according to the standards of the American Society for Testing Materials, has been found to characterize the fibrous layer with the desired properties, and is preferably employed.

A wear-taking layer 6 of viscous material is provided, and is preferably applied as a coating over the base layer 4. The consistency of this viscous material is such that it is slightly and slowly flowable under pressure to render it capable of coalescing after scarring, so that a continuous smooth surface is restored by wear. A bituminous compound, such as a blown California asphalt having a softening point of from 180° to 195° and a penetration of from 12 to 18, also according to the standards of the Society for Testing Materials, is possessed of the desired characteristics, and is preferably used for the coating 6. This coating layer, while solid at ordinary temperatures, is capable of slow flow under pressure, so that the viscous material will coalesce after scarring to restore a uniform smooth surface under the action of continued wear.

We have found that a suitable weight for the coating 6 is about 13 lbs. per 100 square feet of coated area, this weight however may be varied to suit a given set of conditions. If desirable, a coating of this material may be applied to the underside of the treated fibrous layer 4 for added protection. This coating of course may conveniently be made lighter than the upper coating 6; a weight of 9 lbs. per 100 square feet of coated area having been found suitable. The coatings 6 and 7 unite more or less with the saturant of the fibrous layer to provide a traffic sheet of integral mass, and, since the cementing compound of the bonding layer 3 unites the protective layer 7 with the foundation 2, a unitary paving structure is

provided. This unitary construction of the pavement prevents lateral slipping of the traffic sheet and narrowly localizes shocks and stresses.

While the pavement as above described is satisfactory, and itself is far in advance in point of resistance to wear as compared with other types of pavements, it has a tendency to offer resistance to vehicular traffic, and to become slippery when wet. The reasons underlying the first mentioned of these tendencies are not obvious, but the presence of a resistance to trucking is none the less certain as traction tests have proven.

It is believed however that the resistance is due to a flowing out of the viscous material under the pressure of a truck wheel, and a hillng-up of this material ahead of the wheel as it progresses along the surface of the wear-taking layer; the effect being that the truck is constantly having to climb over a small hill in the surface of the layer. In order to overcome this hillng-up tendency, and still not impair the "healing" or surface restoring properties of the wear-taking layer, we have filled the layer 6 with a stiffening material 8. This material is preferably a granular material, such as sand.

By using a sand filled coating, formed from a mixture of 60% asphalt and 40% sand, we have found by actual traction tests that the resistance to a rolling load is much less as compared with a non-filled coating. The starting resistance in both cases is about the same, but, since the periods of starting are very short as compared to the periods of rolling, this fact is of little consequence in practical trucking operations. Furthermore, actual tests show that the sand filling in the coating does not impair its "self-healing" properties, and while the sand might operate in a minor degree to oppose this action, the opposition is not sufficient to be noted in tests under practical conditions.

It is believed that the filling of granular material hardens, or more probably toughens, the viscous material sufficiently to prevent the hillng-up process when a load is rolling. At the same time, the amount of filling material in the coating necessary to accomplish this result is not sufficient to impair its "healing" properties. The sand used in the coating is preferably a hard silica sand of a size which will pass thru a 30 mesh screen and be retained on a 50 mesh screen. It is to be understood however that the nature and size of the granular material, as well as the amount used in the coating, may be varied; the above mentioned specification for this material being set forth merely as an example.

The granular filling material in the wear-taking layer also provides a skid-proof traction surface, which not only greatly increases traction when the surface of the layer becomes wet, but also materially enhances the safety to vehicular traffic. It is believed that the function of the granular material in this respect will be understood without further comment. If desirable, the wear-taking layer may also be given a dusting of finely ground material 9, such as a ground silica sand of a size which passes thru an 80 or 100 mesh screen, and from which some of the dust has been removed. This finishing coating presents a surface which is mildly gritty, say like Double 0 sand paper.

In conclusion it is pointed out that a pavement is provided which is waterproof and decay-proof; which is highly resistant to wear; which is characterized by a certain measure of resilience to render it vibration absorbent and sound deaden-

ing; which offers substantially a minimum of resistance to trucking; and which presents a skid-proof traction surface.

We claim:

- 5 1. A pavement comprising a supporting sub-structure, and a traffic sheet overlying the sub-structure and comprising a fibrous layer coated with a wear-taking layer of viscous material slightly and slowly flowable under pressure and capable of coalescing after scarring so that a continuous surface is restored by wear, the wear-taking layer being filled throughout with a granular stiffening material to prevent the flowable material from hillng-up under a rolling load 10 without impairing the surface restoring properties of the layer.
2. A pavement comprising a supporting sub-structure, and a traffic sheet overlying and adhesively united to the substructure and comprising a fibrous layer saturated with a semi-solid bituminous material to render the traffic sheet 80 slightly and slowly yieldable under impact, said fibrous layer being coated on its upper surface with a bituminous material to form a wear-taking layer solid at ordinary temperatures, but capable of coalescing after scarring, the wear-taking layer being filled throughout with sand to prevent the flowable material from hillng up under a rolling load without impairing the surface restoring properties of the layer. 85

ANDREW H. IRVING. 90  
OWEN H. ROBERTSON.

|    |     |
|----|-----|
| 20 | 95  |
| 25 | 100 |
| 30 | 105 |
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |